

# UNITED STATES PATENT OFFICE.

CHARLES B. DAVIS, OF NEW YORK, N. Y.

## METHOD OF TREATING PEARL BUTTONS OR BLANKS.

1,312,723.

Specification of Letters Patent.

Patented Aug. 12, 1919.

No Drawing.

Application filed October 29, 1917. Serial No. 199,023.

*To all whom it may concern:*

Be it known that I, CHARLES B. DAVIS, a citizen of the United States, residing at New York, in the county of New York and State 5 of New York, have invented certain new and useful Improvements in Methods of Treating Pearl Buttons or Blanks, of which the following is a specification.

This invention relates to a method of 10 treating pearl buttons or the blanks or material from which said buttons are made, for the particular purpose of bleaching or whitening the same, thereby to increase their desirability and value in trade.

15 What is generally known as the "bark," that is the back of the button or blank or shell is usually dark in color, and, showing through the transparent pearl face gives a corresponding tint to the button which is 20 undesirable because the standard perfect button is white. Of course this bark or backing might be bodily removed but this course would have the disadvantage that the button or shell would be weakened. By my 25 invention I propose to remove from this bark or backing the undesirable coloring, and to substitute for it pure white, with the result that the button will be white.

In the practice of my invention I dissolve 30 out part of the calcium carbonate, which is intermixed with the albuminous matter of the bark (chiefly calcium albuminate), and then combine with this exposed albumin, some substance which will give the desired 35 coloring to the finished article.

Assuming that the purpose is to whiten 40 the button or blank I have found that this can be accomplished as follows. I prepare a solution by adding an equal bulk of water to crystallized nitrate of bismuth, which is heated to near the boiling point, whereupon 45 nitric acid is added, drop by drop, until a clear solution results. The rough blanks are immersed in this solution in the cold, or

the finished buttons are embedded face down 45 in paraffin with the bark exposed and the solution flooded on the bark. The action of the solution is allowed to continue until effervescence ceases, (usually about one minute), when the bark will be found to have become 50 bleached and whitened. The articles are now removed from the solution and washed free from acid in cold water. If they are kept in the water over night they become 55 extremely white, from the complete deposition of the bismuth salt. They are next dried and may be polished or otherwise finished as desired. It will be understood that the nitric acid in solution removes the calcium carbonate from the albumin, while the 60 bismuth deposits, both as the sub-nitrate and as an albuminate.

It will be understood that other acids than nitric acid may be employed to keep the bismuth in solution, as for instance, sulfuric or 65 hydrochloric; or organic acids such as tartaric or citric may be used. Likewise, other metals may be substituted for the bismuth. For instance, butter of antimony will effect a similar result by depositing on the mere 70 addition of water. This invention contemplates the removal from the bark of the calcium carbonate and the deposition in place of the removed material of some material having the desired coloring. 75

I claim:

The method of treating pearl buttons or blanks to change the coloring thereof, which consists in treating the blanks or buttons with a solution comprising water and crystallized nitrate of bismuth, to which has been added nitric acid until a clear solution results, then after the calcium carbonate of the bark has been removed by the nitric acid and replaced by the bismuth, washing 85 the buttons free from acid and drying.

In testimony whereof I affix my signature.  
CHARLES B. DAVIS.

Copies of this patent may be obtained for five cents each, by addressing the "Commissioner of Patents,  
Washington, D. C."